

(No Model.)

S. E. MOWER.

METHOD OF TEMPERING METAL.

No. 337,979.

Patented Mar. 16, 1886.

Fig:1.



Fig:2.



Fig:3.



Witnesses.

Arthur B. Johnson.

John F. C. Prentiss.

Inventor.

Samuel E. Mower.

by Crowley & Gregory atty

# UNITED STATES PATENT OFFICE.

SAMUEL E. MOWER, OF NEW HAVEN, ASSIGNOR TO HENRY G. THOMPSON, OF MILFORD, AND HARRY G. THOMPSON, OF NEW HAVEN, CONNECTICUT, AND ARTHUR G. THOMPSON, OF NEW YORK, N. Y.

## METHOD OF TEMPERING METAL.

SPECIFICATION forming part of Letters Patent No. 337,979, dated March 16, 1886.

Application filed August 31, 1885. Serial No. 175,738. (No Specimens.)

*To all whom it may concern:*

Be it known that I, SAMUEL E. MOWER, of New Haven, county of New Haven, and State of Connecticut, have invented an Improvement in Methods of Tempering Metal, of which the following description, in connection with the accompanying drawings, is a specification, like letters on the drawings representing like parts.

10 My invention has for its object to effect the partial hardening or tempering of steely metal, either in the form of a strip or of a manufactured article.

15 My invention consists of a method of hardening or tempering steely metal, which consists in drawing the hot metal to be hardened or tempered between asbestos or other non-combustible packing while the edge of the metal to be tempered is kept in or acted upon 20 by the tempering fluid, the said packing preventing the passage of the tempering fluid upon the metal above the said packing, substantially as will be described.

25 In accordance with my invention I have provided a reservoir to contain water or other fluid, the said reservoir having an auxiliary chamber communicating with the reservoir proper, and herein I have shown the said chamber as semicircular in form and covered 30 by metal plates, which are provided with a packing of asbestos, or it may be other equivalent non-combustible material, against which bears snugly the metal as the latter is drawn through the fluid, thereby preventing the said 35 fluid from reaching the metal above the packing.

40 I have also, in accordance with my invention, rigidly fastened one of the said plates to the reservoir, and have provided the other plate, which projects over the side of the reservoir, with slots, through which screws are extended into the frame of the said reservoir, and have secured to the side of the reservoir 45 springs, which act against the projecting edge of the slotted plate, the said spring being of sufficient strength to firmly press the said plate and its asbestos packing against the metal to be tempered.

As heretofore practiced, metal strips have

been either completely tempered by immersing 50 the entire strip in the water, or they have been partially tempered by drawing one edge of the strip against a moistened or wet absorbent band, as in application, Serial No. 175,130.

55 Figure 1 is a top view of apparatus devised by me for tempering bands in accordance with my invention; Fig. 2, a section of Fig. 1 on the line  $x-x$ ; and Fig. 3 shows a piece of metal, the dart lines indicating the extent to which the metal is hardened or tempered.

60 The reservoir A, of metal or any other suitable material, is shown as having its top plate convexed at  $a$  to form an auxiliary chamber,  $a'$ , which communicates with the main chamber B by means of the openings  $c$ . Upon the 65 top of the reservoir A, I have rigidly fastened the plate C by means of the screws S, the said plate being extended to near the central line of the reservoir, where its edge is cut away or made oblique, as at  $c'$ . The plate C', placed 70 at the other side of the central line referred to, is provided with slots  $b$ , (see Fig. 1,) through which screws S' are extended and screwed to the reservoir A, the said plate being extended beyond the said reservoir, 75 where it is acted upon by springs S', (see Fig. 2,) fastened to the said reservoir by the screws S'.

80 The plates C C' are each provided at their edges, near the center of the auxiliary chamber  $a$ , with asbestos or other non-combustible material  $n$ , which is herein shown as packed in slots in the said plates; but it is obvious the same might cover the said plates and be secured thereto in any suitable or convenient 85 manner, the asbestos packing fitting the metal strip D closely, and serving to keep the water from reaching the said metal strip above the said packing as the said metal strip is drawn through the water or other usual tempering fluid below the said packing.

90 In the operation of my improved apparatus the metal strip D, (herein shown as a toothed strip,) after being heated to the required heat for tempering, is run from the furnace (not shown) between the asbestos or non-combustible packing held by the plates C C', the lower edge of the said strip dipping into the said

water or other tempering-fluid in the auxiliary chamber  $a'$ .

It is obvious that various forms of apparatus might be used in connection with the asbestos packing, and I do not limit my invention to the special apparatus described.

In Fig. 3 the heavy or shade lines, ascending above the toothed edge of the strip, indicate the depth to which the metal is hardened, leaving the remainder of the metal comparatively unhardened or soft.

I claim--

The herein-described method or process of hardening or tempering steely metal, which

consists in passing heated metal through water or other fluid between a packing of asbestos or other non-combustible material, whereby the said fluid is prevented from reaching the metal above the packing, thereby tempering only a part of the said metal, substantially as described.

In testimony whereof I have signed my name to this specification in the presence of two subscribing witnesses.

SAMUEL E. MOWER.

Witnesses:

HENRY G. THOMPSON,  
TH. B. CANNON.